

Feb. 11, 1930.

J. H. UHRIG

1,746,373

CENTRIFUGAL PIPE MOLD

Filed June 8, 1927



Inventor

John H. Uhrig

by Francis J. Chaudhury

his Attorney

## UNITED STATES PATENT OFFICE

JOHN H. UHRIG, OF BEVERLY, NEW JERSEY, ASSIGNOR TO UNITED STATES CAST IRON PIPE & FOUNDRY COMPANY, OF BURLINGTON, NEW JERSEY, A CORPORATION OF NEW JERSEY

## CENTRIFUGAL PIPE MOLD

Application filed June 8, 1927. Serial No. 197,273.

My invention relates to steel molds used in the centrifugal casting of cast iron pipes by the De Lavaud method. These molds are generally made from steel forgings and have 5 their inner face highly finished, preferably polished, and their useful life is generally ended by the development of deep cracks on their inner surfaces, generally at the end of the mold into which the molten iron is first 10 introduced, which in the case of bell ended pipe is the bell end of the mold, which bell end is for other reasons exposed to greater strains than the cylindrical portion of the mold.

15 I have found by examination of large numbers of used molds that circumferential and longitudinal hair line cracks on the inner polished surface of the steel molds develop early in their use and that where these surface cracks are symmetrically and comparatively closely developed so as to break the inner surface into small rectangles and give it a somewhat alligator skin-like appearance, the mold will usually have a longer useful 20 life and injurious cracks will be slower to appear.

The object of my invention is to provide 25 a mold in which the development of symmetrical hair line cracks will be promoted and in which also the smooth surface of the mold, or of such zones of the mold as are most likely to fail in use, will be microscopically roughened without impairing to sight or touch the smooth surface and thus, as I 30 believe, providing for a less intimate contact of the molten metal with the mold surface and slightly slowing the transmission of heat from the molten metal to the body of the mold.

40 For the best results I have found that a method of roughening the smooth surface of the mold which will at the same time harden the inner skin is highly desirable and 45 I have discovered that this can best be obtained by sand blasting the surface with spherical shot preferably of steel. Good results can however be obtained by the use of the ordinary sand blast or by etching the 50 smooth surface to produce a microscopic

roughening though such treatments do not harden the roughened surfaces.

My invention consists in the provision of a smooth steel mold having its smooth surface microscopically roughened and preferably hardened in zones where injurious cracks are liable to occur.

In the drawings:

Figure 1 is a sectional view of a bell ended steel mold showing its inner polished surface 60 broken up into rectangles by fine hair line cracks which develop in use, and

Figure 2 is a rough indication of a portion of the mold surface enormously magnified to show the hardened and microscopically 65 roughened polished surface.

A is the mold; A<sup>1</sup> its bell end; A<sup>2</sup> its smooth inner surface; B and C the circumferential and longitudinal hair line surface cracks which develop in the use of the best 70 molds. E, Fig. 2, indicates the hardened skin of the polished surface and F indicates the microscopic roughening of the surface.

It will be understood that my molds are prepared in the usual way and treated after 75 finishing to microscopically roughen or harden and roughen the highly finished surface in zones where destructive cracks are most likely to occur in use.

Having now described my invention, what 80 I claim as new and desire to secure by Letters Patent is:

1. A steel mold for the centrifugal casting of cast iron pipes having its inner surface highly finished and in parts microscopically roughened after polishing.

2. A steel mold for the centrifugal casting of cast iron pipes having its inner surface highly finished and in parts surface hardened and microscopically roughened 90 after finishing.

JOHN H. UHRIG.